

## UNITED STATES PATENT OFFICE

SAMUEL ISIDORUS VLES, OF ARNHEM, NETHERLANDS

PROCESS OF PREPARING ARTIFICIAL TEXTILE PRODUCTS WITH REDUCED LUSTER  
FROM CELLULOSE COMPOUNDS

No Drawing. Application filed September 21, 1927, Serial No. 221,150, and in the Netherlands May 28, 1927.

My present invention relates to a process of preparing artificial textile products with reduced luster (desirable for special purposes) from cellulose compounds such as commonly used in spinning according to the so called dry or evaporative method in which a solution of a cellulose compound in a volatile solvent is extruded through fine apertures or orifices into an atmosphere in which the volatile solvent is evaporated.

In my present specification and claims the expression "cellulose compounds" is intended to cover only such cellulose compounds which are, by dryspinning, converted into filaments due to the evaporation of the volatile solvent. As examples of solutions of cellulose compounds which I may use the following are given: cellulose acetate, cellulose nitrate, nitro-acetyl cellulose, alkyl-, aryl-, or aralkyl ethers of cellulose, in acetone, ether, alcohol-ether, acetic acid and other mixed or non-mixed ethers or esters of cellulose in volatile solvents or mixtures of solvents.

In order to obtain a wool-like product from cellulose acetate it has already been proposed to treat the product, in the form of hanks, with warm or boiling water, solutions of ammonium, potassium, or calcium rhodanide, etc. One disadvantage of this method lies in the fact that a special after-treatment of the finished spun product and also washing and drying are necessary. Further disadvantages are that the spun product becomes too wool-like, and that the hanks shrink and often become intermingled.

The object of my present invention is to provide a process whereby it is possible to obtain artificial textile products with reduced luster from cellulose directly (i. e. without any after-treatment and also to obtain any degree of reduction of the luster.

According to my invention the said result is obtained by carrying out the spinning process in the presence of water, which term also includes water vapour, in the use of the so called drying or evaporative method.

My invention may be realized in different ways. A sufficient amount of water may be maintained in the spinning cell, and the spun material may be introduced, before the

threads are wholly deprived of the solvent, into a second room in which sufficient water vapour is present.

Further, the object in view may be attained by using a spinning solution to which water has been added and of which the viscosity has been brought back to the normal. 55

In order that my invention may be clearly understood, the following example of a solution of cellulose acetate in acetone will now 60 be described.

The solution of cellulose acetate in acetone is introduced into a spinning cell in a downward direction, through fine apertures, the spun material being led along a thread guide to the winding apparatus. The spinning process is carried out in the presence of water or, alternatively, in the presence of 65 water vapour.

The spinning process may be carried out in 70 such a way that water vapour is present in the spinning cell, the amount of water vapour increasing with the rise of temperature.

Alternatively, water vapour is not introduced into the spinning cell, the spun material being led out of the spinning cell before the solvent is completely removed, and being then led into a room in which water vapour is present. 75

I may, for example, use a second cell or 80 the winding apparatus may be arranged in a moist atmosphere or the spun material may be freed from the acetone in a room in which water vapour is present, during its travel from the spinning cell to the winding apparatus. 85

The product obtained will be more or less dull, the degree of dullness depending upon the length of the way over which the spun material is led into the damp atmosphere and 90 also upon the degree of humidity and the temperature of the air.

A small proportion of water may also be added to the spinning solution, the proportion of water depending amongst other things, 95 upon the degree of dullness which is desired to be attained and upon the temperature in the spinning cell.

In general, a greater amount of water must be added if a duller product is desired, and a 100

higher temperature in the spinning cell requires a larger addition of water to the spinning solution.

As the viscosity of the spinning solution decreases by the addition of water, more viscous spinning liquids are preferably used, so that after the addition of the water the viscosity becomes normal again.

Beginning with a spinning solution of normal viscosity, the latter may be restored by the addition of a substance which increases the viscosity, as well as of water.

Thus, for example, a solution of 13 kg. of cellulose acetate in 100 litres of acetone is prepared, and 2½ litres of water are added thereto. The viscosity decreases, for instance, from 80 to 20 (measured by the aid of a falling glass ball), and by the addition of 5 litres of benzene the viscosity of 80 is restored.

Thereafter, the solution is spun in a spinning cell, in which a temperature of 30°-40° C. prevails, whereby a dull silk is obtained. If the temperature is raised to 40°-50° C. the silk becomes glossy, so that more water has to be added, and, in order to maintain the same viscosity, also more benzene.

Finally, several of the methods described above may be combined by regulating the moisture contained in the air in connection with the water contained in the spinning solution. The more humid the air in the spinning cell, the less water is required to be added to the spinning solution, at the same temperature of the spinning cell.

From the above it will be clear that owing to the large number of variable factors, my present process for the preparation of artificial silk with reduced luster, may be regulated within very wide limits, thus enabling under any circumstance, the most favourable conditions possible to be chosen, which is a great advantage of my said process. Furthermore, it is unnecessary to make any alterations in the apparatus, and, in contradistinction to the known process referred to above no special after-treatment is necessary.

I claim:

1. A process for the preparation of artificial textile products with diminished luster from cellulose compounds, consisting of dissolving the cellulose compound in a volatile solvent, introducing the solution into a spinning cell, evaporating the volatile solvent therefrom by a spinning action, and leading the spun material into an atmosphere into which a predetermined proportion of water is introduced from outside the spinning cell, the proportion of such water being dependent upon the degree of dullness required in the product.

2. A process for the preparation of artificial textile products with diminished luster from cellulose compounds, consisting of dissolving a solution of the cellulose compound in a volatile solvent, introducing the solution

into a spinning cell, evaporating the greater portion of the volatile solvent therefrom by a spinning action, leading the spun material, together with a modicum of its solvent, into an atmosphere into which a predetermined proportion of water is introduced from outside the spinning cell, the proportion of such water being dependent upon the degree of dullness required in the product.

In testimony whereof I affix my signature.

SAMUEL ISIDOOR VLES.

75

80

85

90

95

100

105

110

115

120

125

130